# EUROPEAN PATENT SPECIFICATION

(11) **EP 0 051 826 B1**
(45) Date of publication and mention of the grant of the patent: **05.02.1986**
(21) Application number: 81109284.0
(22) Date of filing: 29.10.1981
(51) Int. Cl.: H01C 17/26, H01C 17/06, H01C 17/22

(54) **Method of producing thick film resistor element of accurate resistance**
Verfahren zur Herstellung eines genauen Dickschichtwiderstandelements
Procédé de fabrication d'un élément résistif de précision à film épais

(30) Priority: 07.11.1980 JP 155791/80
(43) Date of publication of application: 19.05.1982
(73) Proprietor: NISSAN MOTOR CO., LTD., Yokohama-shi Kanagawa-ken (JP)
(72) Inventor: Akimune, Yoshio, Kanazawa-ku Yokohama City (JP); Uchida, Masaaki, Isogo-ku Yokohama City (JP); Ambe, Satoshi, Yokosuka City (JP)
(74) Representative: TER MEER STEINMEISTER & PARTNER GbR

## Description

### Background of the invention

This invention relates to a method of producing a thick film that serves as a resistive element on an insulating substrate by applying a paste containing a powder of a resistor material onto the surface of the substrate to form a paste layer and then firing the substrate to sinter the resistor material contained in the applied paste, and more particularly to a technique to enhance accuracy of the resistance of the sintered thick film produced by this method.

Thick film resistor elements of the above mentioned type are formed largely as basic elements of hybrid integrated circuits, but also they are utilized in some other electric or electronic devices other than integrated circuits. As a specific example, an oxygen sensor element of the solid electrolyte concentration cell type recently used in automobiles includes a thick film resistor as a heat-generating means for maintaining the sensor element at a desirably elevated temperature.

In the present application the term "thick film" is used in the sense of a film thicker than about 1 pm, as is customary in the current electronic technology. There is no strict upper limit to the thickness of the film. The thickness may reach tens of microns.

A thick film to serve as a resistive element is usually formed by a printing-and-firing method using a paste containing a powder of an electronically conducting resistor material such as a noble metal powder. The first step of this method is to print the paste adjusted to a suitable viscosity onto a major surface of an insulating substrate. Usually a screen-printing method is employed to form a desirably patterned paste layer. After drying of the printed paste layer to evaporate the liquid component of the paste, the substrate is fired so as to achieve sintering of the resistor material contained in the paste layer. The sintered powder of the resistor material constitutes a thick film which may be microscopically porous but adheres firmly to the surface of the substrate.

To obtain a thick film of this category with a resistance value accurately as intended, it is important to strictly control the thickness of the paste layer formed by the screen-printing process. That is, the resistance of the sintered thick film depends greatly on the thickness of the printed paste layer. Therefore, not only the viscosity of the paste but also the pressure exerted on the squeegee of the screen-printing apparatus and the speed of the movement of the squeegee relative to the screen are minutely adjusted so as to form a paste layer of an appropriate thickness. The thickness control at this stage can be accomplished fairly accurately, but in the case of mass production some dispersion of the thickness values is inevitable. Furthermore, the resistance of the sintered thick film is affected considerably by the firing conditions represented by the firing temperature and the duration of firing, and also by the physical state of the printed and dried layer subject to firing. For these reasons, dispersion of the resistance values of the mass-produced thick film resistor elements is considerably large and sometimes reaches about ±20% of the intended value even though the printing process is performed with due control of the thickness. On the other hand, the tolerance of the resistance is rarely larger than ±5%.

With a view to increasing the number of acceptable products in mass production of thick film resistor elements by the printing-and-firing method, it has been put into practice to determine optimum firing conditions for each lot by extracting a small number of samples out of the unfired intermediates given by the printing process, firing these samples under standard firing conditions and measuring the resistance of the sintered thick film of every sample. However, even when the firing conditions are adjusted through such a procedure, the resistance values of the sintered thick film exhibit a dispersion of about ±10% in most cases.

Therefore, a considerable large number of the mass-produced sintered thick film must be picked out as rejects, and the loss of such a large number of products naturally leads to an unwantedly high selling price. Nevertheless, it' is rather impractical to enlarge the tolerance of the resistance because it will result in lowering of the precision of the devices in which the thick film resistor elements are used or will raise the need of modifying the circuit design of such devices.

US-A-3 676 633 discloses the electronic trimming of microelectronic resistors formed on a substrate, so as to either increase or decrease the values thereof without affecting their physical qualities. To effect an increase in ohmic value a heating current is passed through the body of the resistor, which current is applied with a relatively low voltage and a high current density provided by a ratio-frequency oscillator preferably operating to the range of 2000 to 3000 Hz.

### Summary of the invention

It is an object of the present invention to provide an improved method of producing a thick film resistor element, which method fundamentally belongs to the above described printing-and-firing method but, nevertheless, gives a thick film the resistance of which is very close to an intended resistance and, when applied to mass production, can greatly increase the percentage of acceptable products. The method according to the invention of producing a thick film resistor element having a predetermined resistance on an insulating substrate comprises the steps of
(a) applying a paste containing a powder of an electronically conducting resistor material dispersed in a liquid vehicle onto a major surface of the substrate to form a paste layer,
(b) drying the paste layer,
(c) firing the substrate to achieve sintering of the resistor material contained in the paste layer, and then
(d) applying an alternating voltage to the thick film as the product of the firing step so as to increase the resistance of said thick film from a provisional resistance up to a predetermined resistance, and is

characterized in that said steps (a) and (c) are performed in such a way that said thick film as the product of the firing step has always a provisional resistance lower than said predetermined resistance, that said alternating voltage has a very low frequency from about 1/300 Hzto about 1 Hz, and that magnitude of said alternating voltage is more than about two times higher than a maximum voltage applied to the thick film resistor element in practical use thereof but not more than about five times higher than said maximum voltage.

The magnitude of the alternating voltage and the duration of application of the alternating voltage would be selectively determined according to the difference between the predetermined resistance and the provisional resistance.

The application of an alternating voltage to the sintered thick film causes displacement of microscopical voids among the fine crystal grains of the sintered resistor material as the effect of a phenomenon called electromigration and results in partial breaking of the contacts between the crystal grains. Therefore, the effect of this treatment can be regarded as a decrease in the effective cross-sectional area of the sintered thick film, and a resultant increase in the resistance. As will be understood, the resistance of the sintered thick film under this treatment increases as the duration of the treatment is prolonged and as the magnitude of the alternating voltage is raised.

The improvement according to the invention can readily be put into industrial practice without the need of modifying the apparatus and fundamental procedures of the conventional printing-and-firing method and has the effect of enhancing the accuracy of the resistance of the produced thick film resistor elements and greatly increasing the percentage of acceptable products. Therefore, this invention will bring about a considerable reduction of the total production cost and will enable to lower the selling price. Furthermore, this invention is expected to allow automation of the production of thick film resistor elements by a printing-and-firing method.

### Brief description of the drawings

Fig. 1 shows diagrammatically the manner of application of an alternating voltage to a thick film resistor element, which is shown in a sectional view, in an example of the method according to the invention;
. Fig. 2 is a chart showing an exemplary waveform of an alternating voltage used in a method of the invention;
Fig. 3 is a graph showing the degree of increase in the resistance of a thick film resistor element to which an alternating voltage of the characteristic as shown in Fig. 2 was applied for a variable duration in an example of the method of the invention; and
Fig. 4 is a graph similar to Fig. 3 but shows an experimental result in another example of the invention.

### Description of the preferred embodiments

In a method according to the invention, the application of a conducting paste onto a substrate and sintering of the printed and dried paste layer are accomplished by using known techniques. That is, the application of the paste is usually accomplished by a screen-printing method, and the sintering is effected in either air or a non-oxidizing gas atmosphere at a temperature in the range from about 800°C to about 1500°C depending on the kind of the resistor material.

To obtain a sintered thick film having a provisional resistance Rₐ lower than a truly desired resistance Rₛ of the finished thick film, it is necessary to suitably adjust the composition of the paste, viscosity of the paste, thickness of the paste layer given by the printing process and/or the firing conditions. In practice, it will be most suitable to realize the provisional resistance Rₐ primarily by adjusting the thickness of the paste layer because often it is difficult to significantly alter the paste composition and/or the firing conditions without unfavorably affecting the properties of the sintered thick film other than the resistance.

The proportion of the provisional resistance Rₐ to the truly desired resistance Rₛ can be selected in a pretty wide range. However, in most cases it is undesirable to make the provisional resistance Rₐ below 50% of the desired resistance Rₛ because the application of an alternating voltage high in magnitude and long in duration enough to increase such a low resistance Rₐ up to the level of Rₛ tends to cause weakening of the mechanical strength of the sintered thick film or the adhesion strength between the thick film and the substrate. In theory, there arises little problem even if the provisional resistance Rₐ is very close to the desired resistance Rₛ, but from a practical point of view an extremely small difference between these two resistance values Rₐ and Rₛ, for example Rₐ being 99% of Rₛ, will be meaningless. Accordingly the upper limit of Rₐ in the practical sense will be about 90% of Rₛ.

In the case of industrial production of thick film resistor elements, a primary fractor in determining the proportion of the provisional resistance Rₐ to the desired resistance Rₛ is the width of dispersion of the provisional resistance values Rₐ of the actually obtained sintered thick films in comparison with the tolerance of the resistance Rₛ of the final products.

For example, assume that the tolerance of the desired resistance Rₛ is ±2% (that is, resistance values in the range from 0.98Rₛ to 1.02Rₛ are acceptable) and that actual values of the provisional resistance Rₐ exhibit a dispersion of ±20%. In this case, if the provisional resistance Rₐ (as an aimed value or average value) is set at 90% of Rₛ, the actual values of Rₐ will disperse in the range from 0.72Rₛ to 1.08Rs so that a portion of the sintered thick film become above 1.02Rₛ (upper control limit) in resistance. This portion of the intermediate products cannot be remedied and must be picked out as rejects, so that the object of increasing the percentage of acceptable products cannot fully be accomplished even though the intermediates lower in resistance Rₐ than 0.98Rₛ can be rendered acceptable by the voltage application according to the invention. When the aim of the provisional resistance Rₐ is set at 85% of Rₛ, actual values of Rₐ will fall within the range from 0.68Rₛ to 1.02Rₛ. Then the percentage of the finally rejected products becomes almost 0% since the sintered thick films below 0.98Rₛ in resistance can be rendered acceptable by the treatment according to the invention while the remaining portion having resistances of 0.98Rₛ to 1.02Rₛ can be accepted without any treatment. If the dispersion of actual values of the provisional resistance Rₐ can be assumed to be ±10%, a similarly good result can be obtained even by setting the aim of Rₐ at 90% of Rₛ because actual values of Rₐ will not exceed 0.99R_{S}.

Care should be taken also when it is intended to provide a relatively large difference between the desired resistance Rₛ and the provisional resistance Rₐ because in that case there arises a possibility that actual values of Rₐ will become below about 50% of Rₛ. If the tolerance of Rₛ is ±2% and the dispersion of Rₐ is considered to be 20%, it is unsuitable to make the aim of Rₐ as low as 60% of Rₛ because then actual values of Rₐ will range from 0.72Rₛ to 0.48Rₛ, whereas it is difficult to achieve about 100% increase in the resistance (e.g. from 0.48Rₛ to at least 0.98Rₛ) by the treatment according to the invention without unfavorably affecting the mechanical strength of the thick film. When the aim of the provisional resistance Rₐ is raised to 70% of Rₛ, actual values of Rₐ will fall within the range from 0.84Rₛ to 0.57Rₛ and, therefore, it will be possible to increase the resistances of almost all the intermediates of the thick film resistor elements to acceptable values within the range from 0.98Rₛ to 1.02Rₛ without significantly suffering from unfavorable side-effects.

For the above explained reasons, in most cases it is suitable to set the aim of the provisional resistance Rₐ at a value in the range from 70 to 85% of the truly desired resistance Rₛ.

The duration of application of the alternating voltage is usually from several seconds to tens of minutes.

The present invention places no particular restriction on the materials or composition of the conducting paste for forming the thick film. That is, conducting pastes conventionally used to produce thick film resistor elements are all useful in the present invention. As mentioned hereinbefore, the paste is a uniform dispersion of a powdered resistor material in a liquid vehicle, which is usually a solution of an organic polymer in an organic solvent. For example, the resistor material may be a noble metal powder such as silver powder, platinum powder or ruthenium powder or a powder of an alloy of noble metals such as Pt-Rh, Ag-Pd, Au-Pt or Au-Pd. To adjust the viscosity of the paste or the resistance of the formed thick film and/or enhancing the adhesion strength of the formed thick film, such a metal or alloy powder may optionally be admixed with a glass frit powder and/or a metal oxide powder such as RuO₂ powder, AI₂0₃ powder or Zr0₂ powder. An example of organic polymers suitable as the binder component of the organic vehicle is a cellulose derivative such as methyl cellulose or ethyl cellulose, and an example or organic solvents suitable to cellulose derivatives is terpineol. The material of the substrate can freely be selected among various ceramic materials. Some examples are alumina, mullite, spinel, silica and forsterite. If desired, it is possible to use a metal substrate having a ceramic coating.

The following examples are presented to illustrate the method according to the invention. Needless to mention, these examples are by no means limitative of the invention.

### Example 1

A platinum paste was prepared by first dissolving 15 parts by weight of an ethyl cellulose resin in 85 parts by weight of a-terpineol to obtain an organic vehicle and then uniformly dispersing 65 parts by weight of a fine powder of platinum in 35 parts by weight of the organic vehicle.

Referring to Fig. 1, this platinum paste was applied onto a major surface of an alumina substrate 10 by a screen-printing method by using a screen patterned correspondingly to the intended pattern of a thick film to be formed. The printed paste layer was dried at a temperature of 100°C for a period of about 1 hr, and thereafter the substrate 10 with the dried paste layer thereon was fired in air at about 1400°C for 2 hr to thereby achieve sintering of the platinum powder contained in the printed paste layer. The sintered platinum powder constituted a thick film resistor element 12 which adhered firmly to the surface of the substrate 10. Indicated at 14 are a pair of conducting leads, which were arranged prior to the firing process such that the two terminals of the sintered thick film resistor element 12 made intimate contact with the two leads 14, respectively.

At the screen-printing stage, the thickness of the printed paste layer was controlled such that, when a large number of samples of the thick film 12 were formed by the same procedure and under the same conditions, the average resistance Rₐ of the sintered thick film became 4.8 ohms. In this example, a truly desired resistance Rₛ of the thick film resistor element 12 was 6.0 ohms, but it was intended to make the actual resistance Rₐ of the sintered thick films about 80% of the truly desired resistance value Rₛ (6.0 ohms).

By measuring the resistance Rₐ of each thick film 12 formed in this example, the following six groups of samples were selected out of the many products.
Group A: Rₐ=3.1 ohms (about 52% of the truly desired value Rₛ)
Group B: Rₐ=3.4 ohms (about 57% of Rₛ)
Group C: Rₐ=4.0 ohms (about 67% of Rₛ)
Group D: Rₐ=5.0 ohms (about 83% of Rₛ)
Group E: Rₐ=5.4 ohms (about 90% of Rₛ)
Group F: Rₐ=5.8 ohms (about 97% of Rₛ)

To each of these samples, an alternating voltage was applied by connecting the leads 14 to an alternating voltage supplying circuit 16, which was fundamentally a combination of a DC power supply 18 and a switching device 20 for periodical changeover of the polarity of the output voltage. The circuit 16 was adjusted such that a square wave alternating voltage of the characteristic shown in Fig. 2 was applied to each sample thick film 12. That is, +10 volts and -10 volts were alternated every one minute. The duration of the application of the alternating voltage was varied from Group to Group of the samples and made longer for the samples of smaller resistance values, and more minutely varied for the individual samples of the same Group. The details of the variations are shown in the following Table 1. After the application of the alternating voltage the resistance of each sample was measured. The resistance values measured at this stage are also contained in Table 1. Assuming that the tolerance of the desired resistance Rₛ is 6.0 ohms ±2% (i.e. in the range from 5.88 to 6.12 ohms), the samples in Table 1 were evaluated as OK when the resistance after the application of the alternating voltage was within this range but otherwise as NG. It was confirmed that the application of the alternating voltage caused an increase in the resistance of each thick film and that the manner of increase in the resistance was as shown in Fig. 3 for the samples of Groups D, E and F.

We have recognized that the application of an alternating voltage to the sintered thick film 12 has an unfavorable effect on the strength of adhesion of the thick film 12 to the substrate 10, presumably as the result of a change in the physical structure of the sintered film 12 attributed to the aforementioned electromigration phenomenon. In this example, the degree of this side-effect of the voltage application was examined by the following test method.

The above described platinum paste was applied onto the alumina substrate 10 by screen-printing in a rectangular pattern (20 mmx5 mm), and a cylindrical rod (not illustrated) of alumina having a diameter of 2 mm was vertically placed on the printed paste layer. The substrate was fired in this state at 1400°C for 2 hr to complete the formation of the thick film 12 which adhered to both the substrate 10 and the alumina rod. This thick film was so formed as to have the same thickness as the thick films 12 in the samples subjected to the above described resistance-increasing treatment. A number of samples were produced by this procedure, and a portion of these samples were subjected to an adhesion strength test in which the alumina rod was pulled until separation of the thick film from the substrate, or separation of the rod from the thick film, to measure the pull force at the moment of beginning of the separation as the peel strength of the thick film. On the average, the peel strength of the tested thick films was 4.4 kg/mm².

The remaining samples were classified into six groups according to the resistance values of-the thick films similarly to the Groups A to F in the foregoing test, and the alternating voltage of the characteristic of Fig. 2 was applied to each sample for a period of time different from sample to sample depending on the initial resistance value, as shown in Table 1. After the application of the alternating voltage, every sample was subjected to the above described strength test. The peel strength values measured in this test are also presented in Table 1. From a practical viewpoint, it is required that the peel strength of the thick film after the resistance-increasing treatment be at least 60% of the initial peel strength value, 4.4 kg/mm². In Table 1, therefore, the samples below 2.64 kg/mm² in the peel strength are evaluated as NG and the others as OK.

As can be seen in Table 1, in this experiment it was impossible to obtain fully practicable thick film resistor elements from the samples of Group A, because the application of the alternating voltage for a very long period of time to increase the resistance by nearly 100% (the initial resistance Rₐ was about 52% of the desired resistance Rₛ, 6.0 ohms) caused a great decrease in the peel strength of the thick film. For the samples of Groups B-F (i.e. when the initial resistance Rₐ was above 56% of the desired resistance Rₐ), it was possible to realize the desired resistance Rₛ (considering the tolerance of ±2%) with the maintenance of an acceptable peel strength by adequately determining the duration of the application of the alternating voltage. The thick film resistor elements produced in this example were intended to be used with the application of a voltage not higher than 3 volts. This means that the magnitude of the voltage used in the resistance-increasing treatment was more than three times as high as a maximum voltage during use of the thick film resistor elements. Therefore, there is little possibility that the resistance of the thick film resistor elements after the treatment will further increase during practical use thereof.

By further experiments, it was confirmed that the fraction defective after the resistance-increasing treatment can be made less than 5% even when the tolerance of the resistance is as strict as ±2%. This is a surprising improvement because in the case of aiming at the acceptable resistance range of Rₛ ±2% without using the method of the invention about 50% of the products should be rejected.

The square wave alternating voltage used in this example is merely exemplary. It is also possible to use an alternating voltage of a different waveform such as sine wave or sawtooth wave.

### Example 2

A commercially available conducting paste (DuPont's No. 9051 paste) containing a silver-palladium powder was applied onto the alumina substrate 10 by the same screen-printing method as in Example 1. The thickness of the printed paste layer was controlled so as to obtain a thick film having a resistance Rₐ of 4.8 ohms. This resistance value Rₐ was 80% of a truly desired resistance Rₛ, 6.0 ohms. The printed paste layer was dried at a temperature of 100°C for a period of 1 hr, and thereafter the substrate with the dried paste layer thereon was fired at about 900°C for 1 hr to thereby achieve sintering of the Ag-Pd powder contained in the printed paste layer. The sintered Ag-Pd powder constituted a thick film resistor element 12 which adhered firmly to the surface of the alumina substrate 10. The leads 14 in Fig. 1 were provided in the same manner as in Example 1.

By measuring the resistance Rₐ of each thick film formed by the above procedure, the following five groups of samples were selected out of the many samples produced by the same method and under the same conditions.
Group G: Rₐ=3.2 ohms (about 53% of the truly desired value Rₛ)
Group H: Rₐ=3.4 ohms (about 57% of Rₛ)
Group I: Rₐ=4.5 ohms (about 75% of Rₛ)
Group J: Rₐ=5.0 ohms (about 83% of Rₛ)
Group K: Rₐ=5.8 ohms (about 97% of Rₛ)

To each of these samples, an alternating voltage was applied by using the apparatus 16 described in Example 1. The characteristic of the alternating voltage was as shown in Fig. 2, but in this example the amplitudes of the voltage were ±7 volts. That is, +7 volts and -7 volts were alternated every one minute. The duration of the application of the alternating voltage was varied from Group to Group of the samples, and also from sample to sample in the same Group. The details of the variations are shown in Table 2, together with the resistance of each sample measured after the application of the alternating voltage. The criterion for evaluation of the resistance values after the application of the alternating voltage was the same as in Example 1. Fig. 4 shows the relationship between the duration of the voltage application in this example and the extent of increase in the resistance of the thick films of the Groups I, J and K samples. The influence of the resistance-increasing treatment on the adhesion strength of the thick film was examined by the peel strength test described in Example 1, and Table 2 contains evalution of the peel strength after the resistance-increasing treatment on the same criterion as in Example 1. The thick film resistor elements produced in this example were intended to be used with the application of a voltage not higher than 3 volts.

As can be seen in Table 2, in this experiment it was impossible to obtain fully satisfactory thick film resistor elements from the samples of Group G in which the initial resistance Rₐ was only about 53% of the desired resistance Rₛ, 6.0 ohms. For the samples of Groups H-K (i.e. when the initial resistance Rₐ was in the range from about 56% to about 97% of Rₛ), it was possible to realize the desired resistance Rₛ (considering the tolerance of ±2%) with the maintenance of an acceptable peel strength by appropriately determining the duration of application of the alternating voltage. However, in the case of industrial production it is important to determine the nominal value of the initial or provisional resistance Rₐ with due consideration of the width of dispersion of actual values of Rₐ, as explained hereinbefore.

## Claims

1. A method of producing a thick film resistor element having a predetermined resistance on an insulating substrate, the method having the steps of
(a) applying a paste containing a powder of an electronically conducting resistor material dispersed in a liquid vehicle onto a major surface of the substrate to form a paste layer,
(b) drying the paste layer,
(c) firing the substrate to achieve sintering of the resistor material contained in the paste layer, and then
(d) applying an alternating voltage to the thick film as the product of the firing step so as to increase the resistance of said thick film from a provisional resistance up to a predetermined resistance,
characterized in that said steps (a) to (c) are performed in such a way that said thick film as the product of the firing step has always a provisional resistance lower than said predetermined resistance, that said alternating voltage has a very low frequency from about 1/300 Hz to about 1 Hz, and that the magnitude of said alternating voltage is more than about two times higher than a maximum voltage applied to the thick film resistor element in practical use thereof but not more than about five times higher than said maximum voltage.

2. The method according to claim 1, characterized in that said provisional resistance is in the range from about 50% to about 90% of said predetermined resistance.

3. The method according to claim 2, characterized in that said provisional resistance is in the range from about 70% to about 85% of said predetermined resistance.

4. The method according to claim 2, characterized in that the magnitude of said alternating voltage and the duration of application of said alternating voltage being selectively determined according to the difference between said predetermined resistance and said provisional resistance.

5. The method according to claim 1 or 2, characterized in that the thickness of said paste layer is controlled such that said thick film has said provisional resistance.

6. The method according to claim 1 or 2, characterized in that said paste is applied to said substrate by a screen-printing technique.

7. The method according to claim 1, characterized in that said resistor material is a noble metal.

8. The method according to claim 1, characterized in that said resistor material is an alloy of noble metals.

9. The method according to claim 7 or 8, characterized in that said paste additionally contains at least one metal oxide powder.

10. The method according to claim 8 or 9, characterized in that said paste additionally contains a glass frit powder.

11. The method according to claim 1, characterized in that said substrate is formed of a ceramic material.

## Patentansprüche

1. Verfahren zur Herstellung eines Dickfilm-Widerstandselements mit einem vorbestimmten Widerstand auf einem isolierenden Substrat mit den Schritten
(a) Aufbringen einer Paste, die ein Pulver eines elektronisch leitenden Widerstandmaterials in einem flüssigen Vehikel dispergiert enthält, auf eine Hauptoberfläche des Substrates unter Ausbildung einer Pastenschicht,
(b) Trocknen der Pastenschicht,
(c) Brennen des Substrats zum Sintern des in der Pastenschicht enthaltenen Widerstandsmaterials und dann
(d) Anlegen einer Wechselspannung an den als Produkt der Brennstufe gebildeten Dickfilm zur Steigerung des Widerstands des Dickfilms von einem vorläufigen Widerstand auf einen vorbestimmten Widerstand, dadurch gekennzeichnet,
daß die Schritte (a) bis (c) in der Weise durchgeführt werden, daß der als Produkt der Brennstufe gebildete Dickfilm stets einen vorläufigen Widerstand besitzt, der niedriger ist als der vorbestimmte Widerstand,_daß die Wechselspannung eine sehr niedrige Frequenz von etwa 1/300 Hz bis etwa 1 Hz aufweist und daß die Stärke der Wechselspannung mehr als zwei mal so groß ist als die bei der praktischen Verwendung an das Dickfilm-Widerstandselement angelegte Maximalspannung, jedoch nicht mehr als etwa fünf mal so groß als diese Maximalspannung.

2. Verfahren nach Anspruch 1, dadurch gekennzeichnet, daß der vorläufige Widerstand im Bereich von etwa 50% bis etwa 90% des vorbestimmten Widerstands liegt.

3. Verfahren nach Anspruch 2, dadurch gekennzeichnet, daß der vorbestimmte Widerstand im Bereich von etwa 70% bis etwa 85% des vorbestimmten Widerstands liegt.

4. Verfahren nach Anspruch 2, dadurch gekennzeichnet, daß die Stärke der Wechselspannung und die Dauer des Anlegens der Wechselspannung selektiv in Abhängigkeit von der Differenz zwischen dem vorbestimmten Widerstand und dem vorläufigen Widerstand ausgewählt werden.

5. Verfahren nach Anspruch 1 oder 2, dadurch gekennzeichnet, daß die Dicke der Pastenschicht derart gesteuert wird, daß der Dickfilm den provisorischen Widerstand erlangt.

6. Verfahren nach nach Anspruch 1 oder 2, dadurch gekennzeichnet, daß die Paste mit Hilfe der Siebdrucktechnik auf das Substrat aufgebracht wird.

7. Verfahren nach Anspruch 1, dadurch gekennzeichnet, daß das Widerstandsmaterial ein Edelmetall ist.

8. Verfahren nach Anspruch 1, dadurch gekennzeichnet, daß das Widerstandsmaterial eine Edelmetallegierung ist.

9. Verfahren nach Anspruch 7 oder 8, dadurch gekennzeichnet, daß die Paste zusätzlich mindestens ein Metalloxidpulver enthält.

10. Verfahren nach Anspruch 8 oder 9, dadurch gekennzeichnet, daß die Paste zusätzlich ein Glasfrittepulver enthält.

11. Verfahren nach Anspruch 1, dadurch gekennzeichnet, daß das Substrat aus einem Keramikmaterial gebildet wird.

## Revendications

1. Procédé de fabrication d'un élément résistif à film épais ayant une résistance prédéterminée sur un substrat isolant, le procédé comprenant les étapes de
(a) appliquer une pâte contenant une poudre d'un matériau résistif électroniquement conducteur dispersé dans un véhicule liquide sur une surface majeure du substrat pour former une couche de pâte,
(b) sécher la couche de pâte,
(c) cuire le substrat pour obtenir la concrétion du matériau résistif contenu dans la couche de pâte, et ensuite
(d) appliquer une tension alternative au film épais en tant que produit de l'étape de cuisson afin d'augmenter la résistance dudit film épais d'une résistance provisoire à une résistance prédeterminée,
caractérisé en ce que lesdites étapes (a) à (c) sont accomplies de façon que ledit film épais en tant que produit de l'étape de cuisson ait toujours une résistance provisoire plus faible que ladite résistance prédéterminée, que ladite tension alternative ait une très basse fréquence d'environ 1/300 Hz à environ 1 Hz et que la grandeur de ladite tension alternative soit supérieure à environ deux fois une tension maximum appliquée à l'élément résistif à film épais dans son usage pratique mais pas plus d'environ cinq fois plus que ladite tension maximum.

2. Procédé selon la revendication 1, caractérisé en ce que ladite résistance provisoire est dans la gamme d'environ 50% à environ 90% de ladite résistance prédéterminée.

3. Procédé selon la revendication 2, caractérisé en ce que ladite résistance provisoire est dans la gamme d'environ 70% à environ 85% de ladite résistance prédéterminée.

4. Procédé selon la revendication 2, caractérisé en ce que la grandeur de ladite tension alternative et la durée d'application de ladite tension alternative sont sélectivement déterminées selon la différence entre ladite résistance prédéterminée et ladite résistance provisoire.

5. Procédé selon la revendication 1 ou 2, caractérisé en ce que l'épaisseur de ladite couche de pâte est contrôlée de façon que ledit film épais ait ladite résistance provisoire.

6. Procédé selon la revendication 1 ou 2, caractérisé en ce que ladite pâle est appliquée audit substrat par une technique d'impression à l'écran.

7. Procédé selon la revendication 1, caractérisé en ce que ledit matériau résistif est un métal noble.

8. Procédé selon la revendication 1, caractérisé en ce que ledit matériau résistif est un alliage de métaux nobles.

9. Procédé selon la revendication 7 ou 8, caractérisé en ce que ladite pâte contient de plus au moins une poudre d'un oxyde de métal.

10. Procédé selon la revendication 8 ou 9, caractérisé en ce que ladite pâte contient de plus une poudre de fritte de verre.

11. Procédé selon la revendication 1, caractérisé en ce que ledit substrat est formé sur un matériau de céramique.
